

1,975,493

Oct 2 1934 XR

1,975,493

6-156

Tx 106/8 ?

UNITE

FICE

105

1,975,493

METHOD AND COMPOSITION FOR  
TREATING TEXTILESWilliam H. Alton, New York, N. Y., and Hilton  
Ira Jones, Wilmette, Ill., assignors to R. T.  
Vanderbilt Co., Inc., New York, N. Y., a corpora-  
tion of New YorkNo Drawing. Application September 10, 1932,  
Serial No. 632,632

## 5 Claims. (Cl. 91—70)

This invention relates to the treatment of all textiles either in the form of the threads or yarn or in the form of the product manufactured by weaving or other operation.

5. The composition, if used with certain textiles, such for instance as rayon or other artificial cellulosic textile materials, may be distributed in the solution which is to be spun in making filaments or threads.

10. One object of the present invention is to secure the delusterizing of artificial silk commonly known as rayon. As an important step in the securing of such delusterizing, we employ a colloidal aluminum silicate which may be either natural or

15. artificial, but is preferably of the bentonitic type such as bentonite. Bentonite will absorb a very large amount of water and will correspondingly increase in volume. After being applied to the fabric the drying will cause corresponding shrink-

20. ing in volume and during the shrinking the minute filaments or fiber ends will be drawn in or caused to closely adhere to the threads so as to make the fabric more sheer. This material, when applied to rayon filaments and dried there-

25. on, has a delusterizing effect, but when used alone is unsatisfactory because it is removed in whole or in part during washing and will spot or become irregularly discolored by the action of water. In connection with the bentonite, we employ salt of

30. a metal which may be dissolved in the bentonite suspension or emulsion and which will react in some way with the bentonite during the drying of the textile to produce a compound which is not water soluble and which acts to delusterize the

35. textile and at the same time to render it waterproof or water repellent. The mixture of bentonite and the metal salt may thus be used with rayon where both delusterizing and waterproofing are desired, or may be used with cotton or other

40. textiles where mere waterproofing or a water repellent character is desired.

If it is desired to dye the fabric, the dye may be dissolved and the metal salt added to this solution, or solutions of the dye and metal salts mixed 45 and mixed with the bentonite so that the dyeing operation takes place in the same bath as that which applies the ingredients going to effect the delusterizing and/or water-proofing.

The metal salt which should be used is prefer- 50 ably one which does not produce any color in the bath or to the fabric unless, of course, the particular color imparted by such metal salt is the one desired. The use of a salt of alumina such as aluminum acetate has been found useful in 55 this process, and the same applies to salts of

the rare-earth metals. In the preparation of metallic salts, the base materials are digested in suitable acids and the insoluble residues strained out. We have found that while these residues are nominally insoluble many of them assume a colloidal form and may be used as a substitute in whole or in part for other colloids.

In addition to the metals above referred to, in some cases we may employ salts of lead, mercury and bismuth.

If it is desired to render the fabric particularly smooth in texture, we may add oleic or stearic acid or fatty acids or softening oils which may be emulsified with the colloidal aluminum silicate prior to the adding of these to the dyeing and waterproofing bath. Materials such as oleic and stearic acid and the like tend to soften the material and make more pliable the yarn or fabric particularly when used as a filling medium for the finish of cotton goods as well as rayon.

In carrying out our process, it is only necessary to use a single bath, and after the treatment of the textile in this bath it may be dried in any suitable manner. The drying results in the formation of the waterproofing compound from the bentonite and the metallic salt and this is primarily upon the outer surface of the threads or filaments, and has a strengthening rather than a weakening effect in addition to its waterproofing action. By making the fibers waterproof, the wet breaking strength of the fibers is very greatly increased.

If the metallic salts used be those of the rare-earth metals, the treatment of the fibers results in not only the delusterizing, dyeing, waterproofing and strengthening, but also the mildew-proofing of the fibers. Among the salts of the rare-earth metals which may be employed, we refer particularly to the acetates of cerium, thorium, lanthanum, or the radio active metals such as uranium or a combination of any of these or of one or more of these with the aluminum, tin or other metallic salts.

The colloidal aluminum silicate is believed to hold the metallic ions of the salt in suspension until after the mixture is brought into contact with the surface of the textile, and is allowed to dry, and the metallic ions apparently enter into combination with the colloidal aluminum silicate and the resulting product is precipitated on to the filaments or fibers and adheres thereto and also bonds together the finer filaments.

Where delusterizing is not important, but the mildew-proofing and waterproofing with or without dyeing is to be secured, we may employ al-

60

65

70

75

80

85

90

95

100

105

110

1975493

OR IN 4271170

bumin either of the vegetable or animal character or may employ emulsifying agents or vegetable colloids such as starches or the milks, saps or juices of fruits, plants, shrubs or trees such as latex from rubber or chicle trees, so-called milk weeds, guayule rubber weed and the like, or mixtures of any of them in combination with suitable forms and quantities of sulphur or other accelerators, vulcanizing agents or curing agents necessary to insure the best results.

As a specific example for dyeing, delusterizing, strengthening, filling, waterproofing and mildew-proofing fabrics at one and the same operation, we may employ the following formula, but other salts than the acetates may be employed and various changes may be made in the ingredients and proportions thereof:

|                    | Parts |
|--------------------|-------|
| Aluminum acetate   | 3     |
| Rare-earth acetate | 1.5   |
| Zinc acetate       | 1.25  |
| Stearic acid       | 0.5   |
| Bentonite          | 1.25  |
| Water              | 200   |

In combination with these ingredients there may be employed the desired amount and character of dye according to the color or shade desired. The parts are given by weight. All of the dye necessary to develop the required shade or color is dissolved in the entire quantity of water to be used and in about twenty parts of this colored water we soak the bentonite until its consistency becomes that of a jelly. Into this jelly we emulsify the previously melted stearic acid and then set temporarily aside as "solution A". We then dissolve the other chemicals into the remaining colored water, this solution being termed "solution B". We then blend solutions A and B and proceed with the usual dyeing treatment, thereafter drying the treated material. This drying results in the metallic ions, in combination with the colloidal material, precipitating on to the filaments of the dyed yarn or fabric and adhering thereto and becoming an integral part thereof.

In our improved process, it will be noted that the usual separate operations of dyeing, waterproofing, mildewproofing and delusterizing are accomplished by the use of a single bath and a single operation.

If rubber latex or aqueous rubber derivatives are employed, they may be used in connection with the bentonite. Where it is desired to soften or size the yarn or fabric, a suitable percentage of cooked starch or gum may be added to the combined A and B solutions or may be used with the B solution alone and in place of the A solution.

Inexpensive cotton fabrics are sometimes "backfilled" which consists of surface application of starch with flour and talc emulsion which is applied hot and then passed through calender rolls to impart a smooth and lustrous finish to remain until the first laundering when it washes out, leaving an open and sleazy looking material, and which, if colored, cannot be restarched because the starch produces a white and smoky

effect over the colored background, and the starch cannot be colored except by an expert.

We have found that a backfilling compound can be made of B solution used with an excess of bentonite and stearic acid with or without the dye solution, and that the bentonite combines with the B solution to form a water resisting compound adhering to the filaments of the fabric to a degree such that the fabric can be laundered or dry cleaned several times with only gradual depletion of the filler.

Bentonite, when used as a backfilling compound, has a waterproofing effect due to the presence of the metallic salts and thus is not readily washed out.

Furthermore, we have found that by the application of more concentrated colloidal solutions of albumin to textiles, such as canvas for example, and then heating these to a temperature of 212° F., the albumin is coagulated upon the textile and in this way the bentonite is held in firm union with the same. A textile treated in this way is found to be very fire resistant. It may be charred by sufficient heat, but it will not glow or flame.

By the term "fibers" or "filaments" as used in 100 this case we include short fibers such as used in paper making as well as the longer fibers used in the textile industry. The process may be employed for waterproofing, mildewproofing and strengthening paper, felt and analogous products as well as textiles. The process may be employed for treating shoe linings, bands of hat, etc.

Having thus described our invention, what we claim as new and desire to secure by Letters Patent is:

1. The method of treating fibers which includes subjecting them to the action of a single bath including a solution of a colloidal aluminum silicate, albumin and salts of one or more rare earth metals, and heating to evaporate moisture and 115 coagulate the albumin.

2. The method of treating rayon fibers, which includes subjecting them to the action of a bath containing bentonite, salts of one or more rare earth metals and albumin, evaporating the moisture, and heating to coagulate the albumin.

3. The process of treating rayon textiles, which consists in subjecting them to the action of a bath containing bentonite, an acetate of one or more rare earth metals and albumin, and heating the 125 solution in the presence of the textile to effect a coagulation of the albumin upon the textile.

4. The process of treating rayon textiles, which includes subjecting the same to the action of a solution containing bentonite, a salt of a rare 135 earth metal, albumin and a compound of the group consisting of oleic or stearic acids, fatty acids and softening oils, and heating the solution in the presence of the textile to effect coagulation of the albumin in the presence of the textile and the other ingredients of the solution.

5. A composition for use in the treatment of textile fibers, which includes bentonite, a salt of a rare earth metal and albumin.

WILLIAM H. ALTON  
HILTON IRA JONES.

50 A flexible composition for filling and filling and waterproofing fabrics and other textile materials, which includes a solution of bentonite, a salt of a rare earth metal, and albumin, and a compound of oleic or stearic acids, fatty acids and softening oils, and heating the solution in the presence of the textile to effect coagulation of the albumin upon the textile and the other ingredients of the solution.

55 The composition may be used in the treatment of fabrics and other textile materials.

80

85

90

95

100

105

110

115

120

125

130

135

140

145

150